

# United States Patent [19]

Sato et al.

[11] 3,925,085

[45] Dec. 9, 1975

[54] DIRECT POSITIVE SILVER HALIDE  
EMULSION

3,767,651 10/1973 Chapman..... 96/101  
3,832,184 8/1974 Sato et al..... 96/101

[75] Inventors: **Akira Sato; Akira Ogawa; Keisuke  
Shiba; Masanao Hinato**, all of  
Kanagawa, Japan

*Primary Examiner*—Won H. Louie, Jr.  
*Attorney, Agent, or Firm*—Sughrue, Rothwell, Mion,  
Zinn & Macpeak

[73] Assignee: **Fuji Photo Film Co., Ltd.,**  
Minami-Ashigara, Japan

[22] Filed: **Dec. 19, 1973**

[21] Appl. No.: **426,145**

## [57] ABSTRACT

### [30] Foreign Application Priority Data

Dec. 19, 1972 Japan..... 47-127574

[52] U.S. Cl. ..... **96/101; 96/107; 96/108;**  
96/130; 96/131; 260/240 E

[51] Int. Cl.<sup>2</sup> ..... **G03C 1/28; G03C 1/16**

[58] Field of Search ..... 96/107, 108, 130, 131,  
96/101; 260/240 E

A direct positive silver halide emulsion containing at least one dimethinecyanine dye wherein the 3-position of a pyrrolo[2,3 b]pyridine nucleus is bonded through a dimethine chain to the 1-, 2-, 3- or 4-position of a cyanine hetero ring nucleus, provided that where the bonding is in the 4-position the cyanine nucleus is a quinoline nucleus or a pyridine nucleus and where the bonding is in the 1- or 3-position the cyanine nucleus is an isoquinoline nucleus.

### [56] References Cited

#### UNITED STATES PATENTS

3,598,595 8/1971 Mee et al..... 96/107

14 Claims, No Drawings

## DIRECT POSITIVE SILVER HALIDE EMULSION

## BACKGROUND OF THE INVENTION

## 1. FIELD OF THE INVENTION

The present invention relates to a silver halide emulsion and, more particularly, it relates to a direct positive silver halide emulsion sensitized with a novel dimethinecyanine dye.

## 2. DESCRIPTION OF THE PRIOR ART

When a silver halide light-sensitive material is exposed to light of wave-lengths to which the light sensitive material is sensitive and is development-processed, the resulting photographic density increases as the exposure amount increases and, ultimately, the photographic density reaches a maximum value. However, when the exposure amount is further increased, the photographic density again is reduced. This phenomenon is generally called solarization. Also, with a silver halide lightsensitive material which has been fogged in an optical or chemical manner in the production of the silver halide emulsion, the same reversal phenomenon (the phenomenon in which the photographic density is reduced with the increase in the exposure amount) as in the case with light is observed. Positive images can be obtained by utilizing the above-described phenomenon.

The term "direct positive silver halide emulsion" as used herein in the invention means a silver halide emulsion prepared so that a positive image can be formed by the usual exposure through a positive original using light followed by development processing.

As sensitizers for conventional negative emulsions, many dyes such as monomethinecyanines, trimethinecyanines, merocyanines, rhodacyanines, and the like are known. However, when these dyes are applied to the sensitization of a direct positive silver halide emulsion, in many cases, a number of defects results, for example, the characteristic curve becomes non-contrasty (or becomes flat) and a re-reversal phenomenon (i.e., a reincrease in the photographic density after the reduction thereof with an increase in the exposure amount) occurs.

In addition, those dyes which have so far been known as sensitizers for direct positive light-sensitive silver halide emulsions have the defect that some of the dye remains (hereinafter "remaining of the dye" or "dye remaining") in the lightsensitive material after processing. Such remaining of dye is inconvenient particularly with photographic papers. Because, when such dyes are used as the sensitizer, a high whiteness cannot be obtained with a black-and-white photographic paper and, with a color photographic paper, true color reproduction becomes impossible. Furthermore, such remaining of the dye is even more inconvenient with a contrasty light-sensitive material, for a copying lithographic type film, an X-ray film, a film for copying microphotographs, and the like.

Dyes which are used for sensitizing direct positive emulsions must not possess any of the above-described defects and must not reduce the maximum density of the image.

## SUMMARY OF THE INVENTION

It is, therefore, an object of the present invention to provide a direct positive silver halide emulsion which provides a high sensitivity, which maintains definite

maximum image density and which does not cause a substantial remaining of dye.

As a result of extensive investigations to attain the above-described objects, the inventors have achieved 5 the present invention. That is, the present invention provides a direct positive silver halide emulsion containing at least one dimethinecyanine dye wherein the 3-position of a pyrrolo[2,3-b]pyridine nucleus is connected to the 1-, 2-, 3- or 4-position of a cyanine hetero 10 ring nucleus (provided that when the 4-position is the bonding position, the cyanine nucleus is a quinoline or a pyridine and when the 1- or 3-position is the bonding position the cyanine nucleus is an isoquinoline) through a dimethine chain, and containing, if desired, 15 an organic desensitizer.

## DETAILED DESCRIPTION OF THE INVENTION

Specific examples of the substituent at 2-position of the pyrrolo[2,3b]pyridine nucleus of the dimethinecyanine dye which is used in the present invention include 20 a lower alkyl group (e.g., having 1 to 4 carbon atoms such as a methyl group, an ethyl group, a butyl group, etc.), an aryl group (e.g., a phenyl group, etc.). A halo- 25 aryl group (e.g., a p-chlorophenyl group, etc.), and a lower alkyl substituted aryl group (e.g., tolyl, etc.).

Specific examples of the cyanine hetero ring nucleus of the dimethinecyanine dye which is used in the invention are, e.g., an oxazoline nucleus, an oxazole nucleus, 30 a benzoxazole nucleus, a naphthoxazole nucleus, a thiazoline nucleus, a thiazole nucleus, a benzothiazole nucleus, a naphthothiazole nucleus, a selenazole nucleus, a benzoselenazole nucleus, a naphthoselenazole nucleus, a 2-pyridine nucleus, a 2-quinoline nucleus, a 4- 35 quinoline nucleus, a benzoimadazole nucleus, an indolenine nucleus, a 3,3-dialkylindolenine nucleus, an imidazo[4,5b]quinoxaline nucleus, a pyrrolidine nucleus, etc. These hetero rings and/or benzene nucleus-fused hetero rings can obtained substituents. Suitable 40 such substituents are, for example, an alkyl group (e.g., a lower alkyl group such as a methyl group, an ethyl group, a propyl group, a butyl group), an aryl group e.g., a lower alkylsubstituted aryl group (e.g., a tolyl group, etc.), a halogensubstituted aryl group (e.g., a p-chlorophenyl group, etc.) a hydroxyl group, an alkoxy 45 group (e.g., a lower alkoxy group such as a methoxy group and an ethoxy group), a carboxy group, an alkoxycarbonyl group (e.g., a lower alkoxy carbonyl group such as a methoxycarbonyl group and an ethoxycarbonyl group), a nitro group, a halogen atom (e.g., a chlorine atom, a bromine atom, a fluorine atom, an iodine atom), and the like.

Specific examples of these cyanine rings are as follows: thiazoles including thiazole, 4-methylthiazole, 4-phenylthiazole, 4-(p-hydroxyphenyl)-thiazole, 5- 55 methylthiazole, 5-phenylthiazole, 4,5-dimethylthiazole, 4,5-diphenylthiazole, and the like; benzothiazoles including benzothiazole, 5-hydroxybenzothiazole, 5-fluorobenzothiazole, 4-chlorobenzothiazole, 5-chlorobenzothiazole, 6-chlorobenzothiazole, 7-chlorobenzothiazole, 7-methylbenzothiazole, 5-methylbenzothiazole, 6-methylbenzothiazole, 5,6-dimethylbenzothiazole, 5-bromobenzothiazole, 6-bromobenzothiazole, 5-phenylbenzothiazole, 6-phenylbenzothiazole, 7-phenylbenzothiazole, 4-methoxybenzothiazole, 5-methoxybenzothiazole, 6-methoxybenzothiazole, 7-methoxybenzothiazole, 5-iodobenzothiazole, 6-iodobenzothiazole, 5-ethoxybenzothiazole, 6-ethoxybenzothiazole, 5-ethoxycarbonylbenzo-

thiazole, tetrahydrobenzothiazole, 5-(N,N-dimethylamido)benzothiazole, 5,6-dimethoxybenzothiazole, 5-hydroxybenzothiazole, 6-hydroxybenzothiazole, 5-nitrobenzothiazole, 6-nitrobenzothiazole, 5-chloro-6-nitrobenzothiazole, and the like; naphthothiazoles including  $\alpha$ -naphthothiazole,  $\beta$ -naphthothiazole,  $\beta,\beta$ -naphthothiazole, 5-methoxy- $\beta$ -naphthothiazole, 5-ethoxy- $\beta$ -naphthothiazole, 7-ethoxy- $\alpha$ -naphthothiazole, 5-hydroxy- $\beta$ -naphthothiazole, 5-ethyl- $\beta$ -naphthothiazole, and the like; oxazoles including oxazole, 4-methyloxazole, 5-methyloxazole, 4-phenyloxazole, 4,5-diphenyloxazole, 4-ethyloxazole, 4,5-dimethyloxazole, 5-phenyloxazole, and the like; benzoxazoles including benzoxazole, 5-chlorobenzoxazole, 5-methylbenzoxazole, 5-phenylbenzoxazole, 6-methylbenzoxazole, 6-nitrobenzoxazole, 5,6-dimethylbenzoxazole, 5-methoxycarbonylbenzoxazole, 5-methoxybenzoxazole, 5-ethoxybenzoxazole, 5-chlorobenzoxazole, 5-methoxybenzoxazole, 5-trifluoromethylbenzoxazole, 5-hydroxybenzoxazole, 6-hydroxybenzoxazole, and the like; naphthoxazoles including  $\alpha$ -naphthoxazole,  $\beta,\beta$ -naphthoxazole,  $\beta$ -naphthoxazole, 7-hydroxy- $\beta$ -naphthoxazole, and the like; selenazoles including selenazole, 4-methylselenazole, 4-phenylselenazole, and the like; benzoselenazoles including benzoselenazole, 5-chlorobenzoselenazole, 5-methoxybenzoselenazole, 5-hydroxybenzoselenazole, tetrahydroxybenzoselenazole, and the like; naphthoselenazoles including  $\alpha$ -naphthoselenazole,  $\beta,\beta$ -naphthoselenazole,  $\beta$ -naphthoselenazole, and the like; thiazolines including thiazoline, 4-methylthiazoline, and the like; 2-quinolines including quinoline, 3-methylquinoline, 6-methylquinoline, 8-methylquinoline, 6-chloroquinoline, 8-chloroquinoline, 8-fluoroquinoline, 6-methoxyquinoline, 6-ethoxyquinoline, 6-hydroxyquinoline, 8-hydroxyquinoline, and the like; 4-quinolines including quinoline, 6-methoxyquinoline, 8-methoxyquinoline, 6-methylquinoline, 8-chloroquinoline, 8-trifluoromethylquinoline, and the like; 1-isoquinolines including isoquinoline, 3-methylisoquinoline, 4-methylisoquinoline, 7-methylisoquinoline, 8-ethylisoquinoline, 6-chloroisoquinoline, 6-methoxyisoquinoline, 8-methox-

dine, 4-chloropyridine, 6-bromopyridine, 4-methoxypyridine, 4-ethoxypyridine, 6-methoxypyridine, 6-ethoxypyridine, 4,6-dimethoxypyridine, and the like; 4-pyridines including pyridine, 2-butylpyridine, 2-decylpyridine, 2-octadecylpyridine, 2,6-dibutylpyridine, 2-benzylpyridine, 2-phenylpyridine, 2,6-diphenylpyridine, 2-chloropyridine, 2-bromopyridine, 2,6-dichloropyridine, 2-methoxypyridine, 2-ethoxypyridine, and the like; imidazo-4,5-b-quinoxalines including 1,3-diethylimidazo[4,5b]quinoxaline, 1,3-dienylimidazo[4,5b]quinoxaline, 1,3-diphenylimidazo[4,5b]quinoxaline, 1,3-diphenylimidazo[4,5b]quinoxaline, 1,3-diallylimidazo[4,5b]quinoxaline, 1,3-dicyclohexylimidazo[4,5b]quinoxaline, and the like; and benzimidazoles including 1-ethylbenzimidazole, 1-ethyl-5-nitrobenzimidazole, 1-ethyl-5,6-dichlorobenzimidazole, and the like.

The above-illustrated dimethinecyanine dyes which is used in the present invention can be synthesized by reacting under heating a pyrrolo[2,3b]pyridine compound aldehyde derivative at 3-position with an alkyl-substituted quaternary ammonium salt of a desired cyanine hetero ring nucleus-containing compound using a molar ratio of about 1:1 in a chemically inert solvent such as acetic acid anhydride, alcohols (e.g., ethanol, isopropanol, butanol, etc.), nitrobenzene, dimethylformamide, acetonitrile, pyridine and morpholine. The solution preferably has a concentration of from about 0.2 to about 1 mol/l. Where acetic acid anhydride is employed as the solvent, it is preferred that the reaction be performed at about 150°C for about 10 minutes and where ethanol is used as the solvent, it is preferred that the reaction be performed at about 80°C for about 10 minutes. Basic catalysts such as basic nitrogen-containing organic compounds (e.g., pyperidine, morpholine, triethylamine, etc.) with pyperidine being preferred. However, it is not necessary to use such a catalyst where acetic acid anhydride is used, since the solvent also functions as a catalyst.

Preferable dimethinecyanine dyes which can be used in the present invention can be represented by the following general formula (I);



isoquinoline, and the like; 3-isoquinolines including isoquinoline, 5-methylisoquinoline, 1-methylisoquinoline, 6-chloroisoquinoline, 6-methoxyisoquinoline, 8-methoxyisoquinoline, and the like; indolenines including indolenine, 3,3-dimethylindolenine, 5-hydroxy-3,3-dimethylindolenine, 3,3-dimethyl-6-chloroindolenine, 3,3,5-trimethylindolenine, 3,3-dimethyl-5-nitroindolenine, and the like; 2-pyridines including pyridine, 4-butylpyridine, 4-decylpyridine, 4-octadecylpyridine, 4,6-dibutylpyridine, 4-benzylpyridine, 4-phenylpyridine, 4,6-diphenylpyridine, 4,6-dinaphthylpyridine, 4-chloropyridine, 4-bromopyridine, 4,6-dichloropyri-

60 wherein R<sub>1</sub> represents a hydrogen atom or a lower alkyl group having 1 to 3 carbon atoms, R<sub>2</sub> represents a hydrogen atom, a lower alkyl group having 1 to 4 carbon atoms or an aryl group, R<sub>3</sub> represents an alkyl group having 1 to 6 carbon atoms, a substituted alkyl group, an allyl group or an aryl group, L<sub>1</sub> represents a methine group, L<sub>2</sub> represents a substituted or unsubstituted methine group (the substituent of L<sub>2</sub> and R<sub>3</sub> can be connected to each other to form a methylene chain), m and n each represents 1 or 2, X<sup>-</sup> represents an anion, and Z represents the non-metallic atoms necessary to complete a cyanine hetero ring nucleus.

$R_2$  and  $Z$  in the general formula (I) above have already been described in detail before.

Specific examples of suitable alkyl groups for  $R_1$  and  $R_2$  include, e.g., a methyl group, an ethyl group, a propyl group, a butyl group, etc., and this alkyl group can further be substituted with a substituent. Preferred alkyl groups for  $R_1$  and  $R_2$  are a methyl group or an ethyl group. Specific examples of alkyl groups having 1 to 6 carbon atoms for  $R_3$  are, for example, a methyl group, an ethyl group, a propyl group, a hexyl group, a hydroxyalkyl group (e.g., a  $\beta$ -hydroxyethyl group, etc.), an alkoxyalkyl group (e.g., a  $\beta$ -methoxyethyl group, etc.), an alkoxyalkyl group (e.g., a  $\beta$ -methoxyethyl group, etc.), a carboxyalkyl group (e.g., a  $\beta$ -carboxypropyl group, etc.), a sulfoalkyl group (e.g., a  $\gamma$ -sulfo-propyl group, etc.), an aralkyl group (e.g., a phenethyl group, a benzyl group, etc.), and the like. Particularly preferable examples of the aryl group for  $R_3$  are, e.g., a phenyl group, a tolyl group, a p-chlorophenyl group and the like.  $R_3$  preferably is a methyl group, an ethyl group or a sulfoalkyl group (e.g., a sulfopropyl group). Specific examples of  $L_2$  include a methine group substituted with, e.g., a lower alkoxyalkyl group (e.g., a methoxyethyl group, a ethoxyethyl group, etc.). This substituent can be connected to  $R_3$  to form a methylene chain. In this case, 5- or 6-membered ring formation is 25 particularly preferable.

Specific examples of  $X^-$  are, for example, a chloride ion, a bromide ion, an iodide ion, a p-toluenesulfonate ion, an ethylsulfonate ion, a perchlorate ion, etc.  $n$  represents 1 when the compound represented by the general formula (I) has a betainelike structure and represents 2 in other cases.

Several specific examples of the compound represented by the aforesaid general formula (I) are illustrated below together with the data for the absorption maximum wave-length ( $\lambda_{max}^{MeOH}$ ) in a methanol solution.



7

 $\lambda_{\text{max}}^{\text{CH}_3\text{OH}} ; 480\text{nm}$  $\lambda_{\text{max}}^{\text{CH}_3\text{OH}} ; 430\text{nm}$  $\lambda_{\text{max}}^{\text{CH}_3\text{OH}} ; 452\text{nm}$  $\lambda_{\text{max}}^{\text{CH}_3\text{OH}} ; 458\text{nm}$  $\lambda_{\text{max}}^{\text{CH}_3\text{OH}} ; 460\text{nm}$ 

8



10

 $\lambda_{\text{max}}^{\text{CH}_3\text{OH}} ; 461\text{nm}$ 

25

 $\lambda_{\text{max}}^{\text{CH}_3\text{OH}} ; 497\text{nm}$ 

40

 $\lambda_{\text{max}}^{\text{CH}_3\text{OH}} ; 420\text{nm}$ 

55

 $\lambda_{\text{max}}^{\text{CH}_3\text{OH}} ; 436\text{nm}$ 

65

 $\lambda_{\text{max}}^{\text{CH}_3\text{OH}} ; 441\text{nm}$



$\lambda_{\text{max}}^{\text{CH}_3\text{OH}}$  ; 444nm



$\lambda_{\text{max}}^{\text{CH}_3\text{OH}}$  ; 451nm



$\lambda_{\text{max}}^{\text{CH}_3\text{OH}}$  ; 447nm

Examples of the synthesis of the compounds which are used in this invention are described below. Unless otherwise indicated all parts, percents, ratios and the like given hereinafter are by weight.

#### SYNTHESIS EXAMPLE 1

##### Synthesis of Dye (1):

10ml of acetic anhydride was added to a mixture of 0.8 g of 1-methyl-2-ethyl-3-formylpyrrolo[2,3b]pyridine and 1.3g of 2-methyl-1-ethylbenzothiazolium iodide and refluxed for about 10 minutes to react. Then, the reaction mixture was cooled with ice-water and the crystal precipitated was collected by filtration. The thus obtained crystal was recrystallized from a methanol-chloroform mixed solvent to obtain 0.6g of dye (1) (m.p.:256°C).

#### SYNTHESIS EXAMPLE 2

##### Synthesis of Dye (8):

20ml of acetic anhydride was added to a mixture of 5 4g of 1-methyl-2-ethyl-3-formylpyrrolo[2,3b]pyridine and 9g of 2-methyl-1,3-diethylimidazo-4,5-b-quinoxalinium p-toluenesulfonate and refluxed for about 10 minutes to react. After cooling, the dye was precipitated with the diethylether and crystallized by adding 10 thereto a sodium iodide aqueous solution and collected by filtration. The thus obtained crystals were recrystallized from a methanol-chloroform mixed solvent to obtain 1.6g of dye (8) (m.p.: 263°C).

Other dimethinecyanine dyes can be synthesized according to the above-described synthesis methods.

It is much more preferable to further incorporate an organic desensitizier in the direct positive emulsion of the present invention.

The organic desensitizier which can be used in the invention is a substance which is capable of capturing free electrons generated in the silver halide grains upon irradiation with radiation and which is adsorbed on the silver halide grains. Further, the organic desensitizier is defined as a substance having a minimum vacant electron energy level which is lower than the electron energy level of the conduction band of the silver halide grains. Preferable desensitizers are compounds having a maximum occupied electron energy level which is lower than the valence electron band of the silver halide grains. The electron energy level of the desensitizer can be measured through complicated procedures are required.

For example, specific examples of determination on extremely symmetric cyanine dyes are given in Tani and Kikuchi; *Photographic Science and Engineering*, vol. 11 (3), p. 129 (1967), and the specific examples of determination on typical merocyanine dyes are given in Shiba and Kubodera; *Pre-print (No. B-12), International Congress of Photographic Science*, 1970 (Moscow). It is known that the electron energy level of these compounds is linearly related to both the anode polarographic half-wave potential ( $E_{ox}$ ) and the cathode polarographic half-wave potential ( $E_{red}$ ).

Many of such organic desensitizers are described in, 45 e.g., U.S. Pat. Nos. 3,023,102; 3,314,796; 2,901,351; 3,367,779; British Pat. Nos. 723,019; 698,575; 698,576; 834,839; 667,206; 748,681; 796,873; 875,887; 905,237; 907,367; 940,152; French Pat. Nos. 1,520,824; 1,518,094; 1,518,095; 1,520,819; 50 1,520,823; 1,520,821; 1,523,626; Belgian Pat. Nos. 722,457; 722,594; Japanese Pat. Publication Nos. 13167/68; 14500/68; and the like.

As the organic desensitizers which can be used in the invention, any of those as described above can be employed. However, particularly preferable results can be provided by compounds which have a cathode polarographic half-wave potential ( $E_{red}$ ) more positive than -1.0 volt and are represented by the following general formula (III);



wherein Z, X<sup>-</sup> and m are the same as defined in the general formula (I), R represents an alkyl group or an allyl group (e.g., having from 1 to 8 carbon atoms, preferably 1 to 4 carbon atoms), and a represents 1 or 2.

Specific examples of R include a methyl group, an ethyl group, a butyl group, a hydroxyalkyl group (e.g., a hydroxyethyl group, etc.), a carboxyalkyl group (e.g., a carboxymethyl group, a 3-carboxypropyl group, etc.), a sulfoalkyl group (e.g., a 2-sulfoethyl group, a 4-sulfobutyl group, etc.), and the like.

Specific organic desensitizers which can be used in the invention are, e.g., phenoxyfranine, pinakryptol yellow, 5-m-nitrobenzylidenerhodanine, 3-ethyl-5-m-nitrobenzylidenerhodanine, 3-ethyl-5-(2,4-dinitrobenzylidene)rhodanine, 5-o-nitrobenzylidene3-phenylrhodanine, 1',3-diethyl-6-nitrothia-2'-cyanine iodide, 4-nitro-6-chlorobenzotriazole, 3,3'-diethyl-6,6'-dinitro-9-phenylthiacarbocyanine iodide, 2-(p-dimethylaminophenyliminomethyl) benzothiazole ethoethylsulfate, Crystal Violet, 3,3'-diethyl-6,6'-dinitrothiacyanine ethylsulfate, 1',3-diethyl-6-nitrothia2'-cyanine iodide, 1,3-diamin-5-methylphenazinium chloride, 4-nitro-6-chlorobenzotriazole, 3,3'-di-p-nitrobenzylthiacarbocyanine bromide, 3,3'-di-p-nitrophenylthiacarbocyanine iodide, 3,3'-dinitrophenylthiacarbocyanine perchlorate, 3,3'-dimethyl-9-trifluoromethylthiacarbocyanine iodide, 9-(2,4-dinitrophenylmercapto)3,3'-diethylthiacarbocyanine iodide, bis(4,6-diphenylpyrryl-2-trimethinecyanine perchlorate, anhydrous 2-p-dimethylaminophenyliminomethyl-6-nitro-3-(4-sulfobutyl)-benzothiazolium hydroxide, 1-(2-benzothiazolyl)-2-(p-dimethylaminostyryl)-4,6-diphenylpyridinium iodide, 1,3-diethyl-5-1,3-neopentylene-6-(1,3,3-trimethyl-2-indolylidene)-2,4-hexadienylidene-2-thiobarbituric acid, 2,3,5-triphenyl-2H-tetrazolium chloride, 2-(4-iodophenyl)-3-(4-nitrophenyl)-5-phenyl-tetrazolium chloride, 1-methyl-8-nitroquinolinium methylsulfate, 3,6-bis-4-(3-ethyl-2-benzothiazolylidene)-2-butenyldiene-1,2,4,5-cyclohexanetetrone, and the like.

As the silver halide emulsions which can be used in the invention, there are, e.g., a silver chloride emulsion, a silver bromide emulsion, a silver chlorobromide emulsion, a silver chloroiodide emulsion, silver iodobromide emulsion, silver chloroiodide emulsion, and the like, as disclosed in U.S. Pat. Nos. 2,401,051; 2,717,833; 2,976,149; 3,023,102; 3,501,306; 3,501,307; 3,501,310 and 3,531,288.

The size of the silver halide grains in these emulsions can be within the range usually employed. However, when the mean grain size is 0.05μ to 1.0μ, preferably 0.2 to 1μ, particularly advantageous results can be obtained. Also, the silver halide grains which can be used in the invention can be either regular grains or irregular grains, though the former provides better effects in the present invention.

Either monodispersed emulsion or monomonodispersed emulsion can be used in the present invention, although the former is more preferable.

In general, original emulsions which can be used for the direct positive silver halide light-sensitive material are classified into the following two groups.

One group of light-sensitive materials are those which have, in the inside of the silver halide crystal, nuclei capable of trapping free electrons, the surface of the silver halide having previously been chemically fogged. This type of emulsion is characterized by the

ability per se to provide a positive image directly. They can be made highly sensitive due to spectral sensitization through the addition of a sensitizing dye and, in addition, the sensitivity in the intrinsic absorption region can be increased. With this type of emulsion, the silver composition must be formulated so that the chemical sensitizer and the salt of Group VIII metal which is used for imparting free electron-trapping nuclei can be absorbed inside the silver halide grains. By the addition of the organic desensitizer, clearing property can be improved and, in particular, "re-reversal" can be prevented. Also, by the addition of bromide ions and iodide ions, the maximum density and sensitivity can be increased and the clearing property can be improved.

Another type of light-sensitive materials for the original emulsions are those which are not provided with free electron-trapping nuclei inside the silver halide grains, the surface of the grains having been chemically fogged. This type of emulsion contains as little lattice defects as is possible and, preferably comprises pure silver bromide regular crystals having no twin plane. This type of emulsion itself provides no direct positive image. However, when an organic desensitizer is adsorbed on the silver halide grains of this emulsion, a direct positive image can be obtained with high sensitivity.

In the present invention, either type of emulsions can be used. In other words, either type of original emulsion can effectively be sensitized by the compound represented by the general formula (I). These emulsions are well known and examples thereof are disclosed in U.S. Pat. Nos. 2,401,051; 2,717,833; 3,976,149; 3,023,102; 3,501,306; 3,501,307; 3,501,310 and 3,531,288.

The silver halide emulsions which can be used in the invention are fogged optically or chemically as disclosed in U.S. Pat. Nos. 2,497,875; 2,588,982; 3,023,102; and 3,367,778. Chemical fogging nuclei are provided by adding a reducing organic compound such as hydrazine derivative, formaldehyde thiourea dioxide, a polyamine compound, an amineborane, methyl-dichlorosilane or the like. In addition, a method of imparting fogging nuclei by the combined use of the reducing agent and an ion of metal more noble than silver (e.g., a gold ion, a platinum ion, an iridium ion, etc.) or, further, a halogen ion can be applied.

In the emulsion which can be used in the present invention, gelatin is mainly used as the protective colloid. Inert gelatin is particularly advantageous. In addition, in place of gelatin, photographically inert gelatin derivatives (e.g., phthaloylated gelatin, etc.), water-soluble synthetic polymers (e.g., polyvinyl acrylate, polyvinyl-alcohol, polyvinylpyrrolidone, polyvinylalginic acid, carboxymethyl cellulose, hydroxymethyl cellulose, etc.), or the like can also be used.

In the direct positive silver halide emulsion of the present invention a fogging nuclei-stabilizing agent (e.g., a mercapto compound, a thione compound, tetrazaindene compound, etc. as disclosed in U.S. Pat. Nos. 2,444,605; 2,444,606; 2,444,607 and 2,444,608), a clearing property-improving agent (e.g., a styrene compound, a triazine compound, etc. as disclosed in U.S. Pat. No. 3,023,102), a brightening agent (as disclosed in U.S. Pat. No. 3,406,070), an ultraviolet absorbant (as disclosed in U.S. Pat. No. 3,434,837), a hardening agent (e.g., chromium alum, a 2,4-dichloro-S-triazine compound, an aziridine compound, an epoxy compound, a mucohalogenetic acid (a halogen formyl

maleic acid compound as disclosed in U.S. Pat. Nos. 3,288,775; 3,017,280 and 2,983,611), a coating aid (e.g., sodium polyalkylenesulfonate, saponin, an anionic surface active agent having a betaine structure, etc. as disclosed in U.S. Pat. Nos. 3,068,101; 3,415,649 and 2,600,831), an antiseptic as disclosed in British Pat. No. 987,010, a plasticizer (e.g., a polyalkyl acrylate, a copolymer of alkyl acrylate and acrylic acid, or a like vinyl polymer, a polyalkylene oxide, etc.), a color coupler as disclosed in U.S. Pat. Nos. 2,376,679; 2,698,794; 3,046,129 and 3,227,554, or like additives can be incorporated.

The amount of the dimethine dye which can be used in the invention cannot be set forth specifically since the amount varies depending upon the amount of silver halide in the emulsion and the surface area of the silver halide grains. However, an amount of about  $1 \times 10^{-6}$  to  $2 \times 10^{-2}$  mol per 1 mol of silver salt provides particularly preferable results. These dyes are used by dissolving in water or a water-miscible solvent such as methanol, ethanol, ethylene glycol monomethyl ether, methyl ethyl ketone, acetone, pyridine, and the like. Ultrasonic vibration can be used for the dissolution of these dyes. Also, methods employed upon sensitizing negative-type emulsions described in, e.g., U.S. Pat. Nos. 3,482,981; 3,585,195; 3,469,987; 3,649,286; 3,485,634; 3,342,605 and 2,912,343, etc. can be used.

The addition of the dyes to an emulsion is conveniently conducted immediately before coating. However, the dyes can be added during chemical ripening or upon formation of the silver halide.

The amount of the organic desensitizer which can be used in the invention cannot be set forth specifically since it also varies depending upon the kind of the desensitizer used. However, the desensitizer is added preferably in an amount of about  $2 \times 10^{-7}$  to  $10^{-1}$  mol per 1 mol of the silver halide.

The emulsion in accordance with the present invention can be applied to various supports to prepare photographic elements. Preferably the thickness ranges from about 5 to  $10\mu$ . The emulsion can be applied to the one side or both sides of the support, which can be either transparent or opaque. Representative examples of supports include a cellulose nitrate film, a cellulose acetate film, a polyvinyl acetal film, a polystyrene film, a polyethylene terephthalate film, and other polyester films, glass, metal, wood, etc. In addition, a support prepared by laminating paper with a plastic can also be used.

The emulsion of the present invention can be suitably processed, after exposure, using the conventionally known processing baths for development, fixation, stabilization, or using a combined processing bath.

A first feature of the present invention is the sensitization of a direct positive silver halide emulsion with a novel dimethine dye having a pyrrolo-2,3-b-pyridine nucleus, which substantially does not cause any remaining of dye.

U.S. Pat. No. 2,323,187 describes that a large amount of sensitizing dye having sensitizing action on conventional negative emulsions, particularly a carbocyanine dye, is effective for the sensitization of direct positive emulsions. However, this method is not preferred since the dye strongly colors the emulsion and results in the dye remaining. On the other hand, British Pat. Nos. 970,621 and 1,186,714 describe that dimethine dyes having a 2-phenylindole nucleus or a 2-

pyridylindole nucleus shows excellent reversal property. However, even such dyes are not satisfactory due to the dye remaining. In addition, when such dyes are added to the direct positive emulsion to the extent that maximum sensitivity is provided, the tendency of the dye to remain becomes particularly great.

The dimethine dyes having a pyrrolo[2,3b]pyridine nucleus of the present invention are characterized in that the remaining of the dye is markedly reduced.

A second feature of the present invention is that the maximum density of the direct positive emulsion is not substantially lowered.

In many cases, dimethine dyes having a 2-phenylindole nucleus, as well as carbocyanine dyes and merocyanine dyes useful for the sensitization of conventional negative emulsions, reduce the maximum density of the direct positive emulsion. The reduction in maximum density occurs during storage with the passage of time as well as immediately after coating the direct positive emulsion. This deterioration of the direct positive photographic light-sensitive material with the passage of time tends to be greater than the deterioration in conventional negative light-sensitive materials. Therefore, removal of this defect has been of great concern. The novel dimethine dye which is used in the present invention shows excellent characteristics in this respect, also.

A third feature of the present invention is that the dimethine dyes which are used in the present invention result in less remaining of the dye and the characteristic curve is not so flat (non-contrasty). In general, a carbocyanine dye or a merocyanine dye useful for the sensitization of a negative emulsion has a strong tendency to have a flattened characteristic curve. This phenomenon of the characteristic curve becoming flat is not preferable for a contrasty direct positive light-sensitive material such as a film for a copying lithographic type film.

Also, the direct positive silver halide emulsion sensitized with the dimethine dye of the invention has the feature that the clearing property (minimum density) is good and "rereversal" phenomenon substantially is not caused.

The novel dimethine dye which is used in the present invention has the excellent characteristics as described above. The reversal sensitivity can be enhanced even more by the combined use of the dye and an organic desensitizer. This combined use enables the production of a direct positive silver halide emulsion having a good clearing property.

The direct positive silver halide emulsion of the present invention can be used for contrasty direct positive silver halide light-sensitive materials such as a light-sensitive material for copying lithographic type films, a light-sensitive material for duplicating original drawings and, in addition, for comparatively non-contrasty direct positive silver halide light-sensitive materials such as a light-sensitive material for copying microphotographs, and a light-sensitive material for copying X-ray photographs. In addition, it can be used for color light-sensitive materials.

The direct positive silver halide emulsion in accordance with the present invention can be exposed using the irradiation of electron beams, X-rays, gamma-rays, etc. as well as the irradiation with light.

The present invention will now be illustrated in greater detail by reference to the following non-limiting examples of preferred embodiments of the invention. Additionally, the dye used for comparison in the examples was the following compound. (A)

15



16

taking the sensitivity of the dye (A) for comparison as 100.

## 5 Composition of the Developer:

|                              |     |   |
|------------------------------|-----|---|
| Metol                        | 3.1 | g |
| Anhydrous Sodium Sulfite     | 45  | g |
| Hydroquinone                 | 12  | g |
| Sodium Carbonate Monohydrate | 79  | g |
| Potassium Bromide            | 2   | g |
| Water to make                | 1   | l |

10

## EXAMPLE 1

First, in order to prepare an original emulsion, Solutions 1 - 4 having the following formulations were prepared.

|                                                |        |    |  |  |
|------------------------------------------------|--------|----|--|--|
| Solution 1                                     |        |    |  |  |
| Inert Gelatin                                  | 8 g    | 20 |  |  |
| An aqueous Solution of Potassium Bromide (1 N) | 5 cc   |    |  |  |
| Water (60°C)                                   | 500 cc |    |  |  |
| Solution 2                                     |        |    |  |  |
| Silver Nitrate                                 | 100 g  |    |  |  |
| Water (60°C)                                   | 500 cc |    |  |  |
| Solution 3                                     |        | 25 |  |  |
| Potassium Bromide                              | 70 g   |    |  |  |
| Water (60°C)                                   | 150 cc |    |  |  |
| Solution 4                                     |        |    |  |  |
| Inert Gelatin                                  | 75 g   |    |  |  |
| Water                                          | 300 cc |    |  |  |

Solution 2 and Solution 3 were added to Solution 1 over a 50 minute period while maintaining the temperature at 60°C and then subjected to physical ripening for 5 minutes. Then, 15cc of a 0.2 N potassium iodide solution was added thereto and the pAg was adjusted to 6.0 using a silver nitrate solution. The pH of the solution was adjusted to 10 using a sodium hydroxide aqueous solution. Then, hydrazine (0.005 millimole per mole of silver halide) and gold chloride (0.005 millimole per mole of silver halide) were added thereto and the ripening was conducted for 10 minutes. After neutralizing with citric acid, the emulsion was washed with water. Then, Solution 4 was added thereto after melting to thereby obtain an original emulsion. The thus obtained emulsion contained regular tetragonal silver halide grains of a mean grain size of about 0.2 which have the crystal face of (100).

To the resulting original emulsion portions were added the dye as set forth and in the amount described in Table 1 and, further, saponin was added (20ml of a 1% solution per kg of emulsion) to the emulsion. Each of the resulting emulsion portions was applied to a cellulose triacetate film in a dry thickness of about 5 microns to obtain samples. Each sample was wedgewise exposed using a 2854°K tungsten light as a light source. Then each of them was development-processed at 20°C for 2 minutes using the following developer and fixed in an acidic hardening and fixing solution. The density was measured using a Model P densitometer made by the Fuji Photo Film Co., Ltd. to obtain characteristic curves. The results of sensitivity, maximum optical density (Dmax) and minimum optical density (Dmin) obtained are shown in Table 1. Additionally, the sensitivity is represented in terms of the reciprocal of the exposure amount necessary for providing a density of

Upon use, this composition was diluted 1:1 by volume with water.

15

TABLE 1

| Sample No. | Dye (molar concentration) cc/100g emulsion | Sensitivity | Dmax | Dmin |
|------------|--------------------------------------------|-------------|------|------|
| 1          | 3 ( $8 \times 10^{-2}$ ) 16                | 1440        | 3.0  | 0.04 |
| 2          | 6 ( $8 \times 10^{-2}$ ) 24                | 500         | 3.0  | 0.04 |
| 3          | 7 ( $8 \times 10^{-2}$ ) 16                | 1580        | 2.9  | 0.04 |
| 4          | 8 ( $8 \times 10^{-2}$ ) 16                | 660         | 3.1  | 0.04 |
| 5          | 10 ( $8 \times 10^{-2}$ ) 16               | 170         | 2.9  | 0.09 |
| 6          | 12 ( $8 \times 10^{-2}$ ) 16               | 416         | 2.9  | 0.05 |
| 7          | 14 ( $8 \times 10^{-2}$ ) 16               | 2080        | 2.8  | 0.04 |
| 8          | A ( $8 \times 10^{-2}$ ) 16                | 100         | 2.4  | 0.23 |

From the results contained in Table 1, it can be seen that, as compared with the dye for comparison, the dye used in the present invention has such excellent properties that it provides a high Dmax, a good clearing property and a high sensitivity.

## EXAMPLE 2

35 First, an original emulsion was prepared in the following manner. Solution 2 (prepared by adding 500cc of water to 100g of silver nitrate and heating to 60°C to dissolve) and Solution 3 (prepared by adding 300g of water to 35g of sodium chloride and heating to 60°C to dissolve) were added to Solution 1 (prepared by adding 5cc of a 1 N sodium chloride solution and 500cc of water to 10g of inert gelatin and heating to 60°C to dissolve) over a 20 minute period under stirring while maintaining the temperature at 60°C. After the completion of the addition, ripening was conducted for 5 minutes. Then, Solution 4 (prepared by adding 200cc of water to 14g of potassium bromide and heating to 60°C to dissolve) was added thereto over a 5 minute period under stirring. Then, ripening was conducted for 10 minutes and, after reducing the temperature, the emulsion was washed with water. Then, it was again heated to dissolve, and the pH was adjusted to 10 followed by adding hydrazine (0.005 millimole per mole of silver halide) and a gold chloride salt (0.005 millimole per mole of silver halide) to ripen for 10 minutes. Thereafter, the pH was adjusted to 6.5 using citric acid. Further, Solution 6 (prepared by adding 300cc of water to 75g of inert gelatin to dissolve) was added thereto to obtain an original emulsion. The thus obtained original emulsion contained silver halide grains of a mean grain size of about 0.15 micron.

60 To the resulting original emulsion portions were added 32cc of a methanol solution of pinakryptol yellow of a molar concentration of  $5 \times 10^{-2}$  and the dye in the amount as set forth in Table 2. Further, mucochloric acid (20ml of a 2% solution per kg of emulsion) and saponin (20ml of a 1% solution per kg of emulsion) were added thereto in suitable amounts. Each of the resulting emulsion portions was applied to a cellulose tri-

acetate film in a dry thickness of about 2 microns to obtain samples.

Each sample was exposed through an optical wedge using as a 2854°K tungsten light as a light source followed by development-processing at 20°C for 3 minutes with a developer having the following formulation and fixing in an acidic hardening and fixing solution.

Composition of the Developer:

|                          |      |    |
|--------------------------|------|----|
| Water (about 30°C)       | 50   | cc |
| Anhydrous Sodium Sulfite | 30   | g  |
| Paraformaldehyde         | 7.5  | g  |
| Sodium Bisulfite         | 2.2  | g  |
| Boric Acid               | 7.5  | g  |
| Hydroquinone             | 22.5 | g  |
| Potassium Bromide        | 1.6  | g  |
| Water to make            | 1    | l  |

The density was measured using a Model P densitometer made by the Fuji Photo Film Co., Ltd. to obtain characteristic curves. D<sub>max</sub> and D<sub>min</sub> were measured in the same manner as described in Example 1 and, in addition, the density of the remaining dye was also measured. This density of the remaining dye was measured by immersing the emulsion-coated sample immediately in the acidic hardening and fixing solution at 20°C for 1 minute and 30 seconds without exposure, washing it with water for 3 minutes, and measuring the density using the above-described densitometer with a blue filter. The results thus obtained are shown in Table 2.

changes and modifications can be made therein without departing from the spirit and scope thereof.

What is claimed is:

1. A direct positive prefogged silver halide emulsion containing at least one dimethinecyanine dye wherein the 3-position of a pyrrolo [2,3b] pyridine nucleus is bonded through a dimethine chain to the 1-, 2-, 3- or 4-position of a cyanine hetero ring nucleus, provided that where the bonding is in the 4-position said cyanine nucleus is a quinoline nucleus or a pyridine nucleus and where the bonding is in the 1- or 3-position said cyanine nucleus is an isoquinoline nucleus, said dimethinecyanine dye being present in an amount sufficient to sensitize said emulsion.

10 2. The direct positive silver halide emulsion as claimed in claim 1, wherein said emulsion contains an organic desensitizer.

3. The direct positive silver halide emulsion as claimed in claim 1, wherein said cyanine hetero ring nucleus is an oxazoline nucleus, an oxazole nucleus, a benzoxazole nucleus, a naphthoxazole nucleus, a thiazoline nucleus, a thiazole nucleus, a benzothiazole nucleus, a naphthothiazole nucleus, a selenazole nucleus, a benzoselenazole nucleus, a naphthoselenazole nucleus, a 2-pyridine nucleus, a 2-quinoline nucleus, a 4-quinoline nucleus, a benzimidazole nucleus, an indolenine nucleus, a 3,3-dialkyindolenine nucleus, an imidazo[4,5b]quinoxaline nucleus, or a pyrrolidine nucleus.

25 4. The direct positive silver halide emulsion as claimed in claim 1, wherein said dimethinecyanine dye is represented by the following general formula (I);



45

TABLE 2

| Sample No. | Dye (Molar Concentration) cc/100g Emulsion | Sensitivity | D <sub>max</sub> | D <sub>min</sub> | Density of Remaining Dye |
|------------|--------------------------------------------|-------------|------------------|------------------|--------------------------|
| 9          | 1 (8 x 10 <sup>-2</sup> ) 24               | 117         | 3.0              | 0.04             | 0.01                     |
| 10         | 3 (8 x 10 <sup>-2</sup> ) 8                | 151         | 3.1              | 0.05             | 0.06                     |
| 11         | 4 (8 x 10 <sup>-2</sup> ) 32               | 257         | 2.9              | 0.04             | 0.01                     |
| 12         | 7 (8 x 10 <sup>-2</sup> ) 8                | 132         | 3.0              | 0.06             | 0.05                     |
| 13         | 14 (8 x 10 <sup>-2</sup> ) 16              | 112         | 3.2              | 0.04             | 0.04                     |
| 14         | 16 (8 x 10 <sup>-2</sup> ) 24              | 115         | 2.8              | 0.04             | 0.01                     |
| 15         | 17 (8 x 10 <sup>-2</sup> ) 24              | 151         | 3.0              | 0.04             | 0.01                     |
| 16         | 20 (8 x 10 <sup>-2</sup> ) 32              | 228         | 2.8              | 0.04             | 0.01                     |
| 17         | A (8 x 10 <sup>-2</sup> ) 16               | 100         | 2.5              | 0.08             | 0.08                     |

From the results contained in Table 2, it can be seen that, as compared with the dye for comparison, the dye used in the invention shows excellent sensitivity, maximum optical density and clearing property and, in addition, causes less remaining of the dye, when used in combination with the organic desensitizer.

While the invention has been described in detail and with reference to specific embodiments thereof, it will be apparent to one skilled in the art that various

50 wherein R<sub>1</sub> represents a hydrogen atom or a lower alkyl group, R<sub>2</sub> represents a hydrogen atom, a lower alkyl group or an aryl group, R<sub>3</sub> represents an alkyl group having 1 to 6 carbon atoms, L<sub>1</sub> represents a methine group, L<sub>2</sub> represents a methine group, wherein said L<sub>2</sub> and R<sub>3</sub> can be connected to each other to form a methylene chain, m and n each represents 1 or 2, X<sup>-</sup> represents an anion, and Z represents the non-metallic atoms necessary to complete a cyanine hetero ring nucleus.

55 5. The direct positive silver halide emulsion as claimed in claim 4, wherein said alkyl group for R<sub>1</sub> is a methyl group, an ethyl group, or a propyl group; wherein said alkyl group for R<sub>2</sub> is a methyl group, an ethyl group, or a butyl group wherein said aryl group for R<sub>2</sub> is a phenyl group, a tolyl group or a p-chlorophenyl group; wherein said alkyl group for R<sub>3</sub> is an alkyl group, a hydroxyalkyl group, an alkoxyalkyl group, a carboxyalkyl group, a sulfoalkyl group, or an aralkyl group; wherein said aryl group for R<sub>3</sub> is a phenyl group, a tolyl group or a p-chlorophenyl group; wherein said methine group for said L<sub>2</sub> is a methine group or a lower alkoxalkyl-substituted methine group, said substituent

being a methoxyethyl group or an ethoxyethyl group and wherein the non-metallic atoms represented by Z form an oxazoline nucleus, an oxazole nucleus, a benzoxazole nucleus, a naphthoxazole nucleus, a thiazoline nucleus, a thiazole nucleus, a benzothiazole nucleus, a

halide emulsion contains a photographic color coupler.

11. The direct positive silver halide photographic emulsion as claimed in claim 2, containing at least one dye selected from the dyes represented by the following general formula (I);



naphthothiazole nucleus, a selenazole nucleus, a benzoselenazole nucleus, a naphthoselenazole nucleus, a 2-pyridine nucleus, a 2-quinoline nucleus, a 4-quinoline nucleus, a benzoimidazole nucleus, an indolenine nucleus, a 3,3-dialkylindolenine nucleus, an imidazo[4,5b]quinoxaline nucleus, or a pyrrolidine nucleus.

6. The direct positive silver halide emulsion as claimed in claim 3, wherein said cyanine hetero ring nucleus is a benzothiazole nucleus, a benzoselenazole nucleus, a benzoxazole nucleus, 3,3-dialkylindolenine nucleus, or an imidazo[4,5b] quinoxaline nucleus.

20 wherein  $R_1$  represents a hydrogen atom or a lower alkyl group,  $R_2$  represents a hydrogen atom, a lower alkyl group or an aryl group,  $R_3$  represents an alkyl group having 1 to 6 carbon atoms,  $L_1$  represents a methine group,  $L_2$  represents a methine group, wherein said  $L_2$  and  $R_3$  can be connected to each other to form a methylene chain,  $m$  and  $n$  each represents 1 or 2,  $X^-$  represents an anion,  $Z$  represents the non-metallic atoms necessary to complete a cyanine hetero ring nucleus, and an organic desensitizer represented by the following general formula (III);

30



40

7. The direct positive silver halide emulsion as claimed in claim 1, wherein said silver halide of said emulsion comprises chemically fogged silver halide grains.

8. The direct positive silver halide emulsion as claimed in claim 7, wherein said silver halide of said emulsion comprises silver halide grains fogged with a reducing agent and a gold compound.

9. The direct positive silver halide emulsion as claimed in claim 7, wherein at least 95% by weight of said fogged silver halide grains have a diameter within about 40% of the mean grain size of said silver halide grains.

10. The direct positive silver halide emulsion as claimed in claim 1, wherein said direct positive silver

wherein  $R$  represents an alkyl group or an allyl group,  $X^-$ ,  $Z$ , and  $m$  are the same as defined above, and  $a$  represents 1 or 2.

45 12. A direct positive silver halide light-sensitive material comprising a support having thereon the direct positive silver halide emulsion as claimed in claim 1.

13. The direct positive silver halide photographic emulsion as claimed in claim 1 wherein the sensitizing amount is within the range of from  $1 \times 10^{-6}$  to  $2 \times 10^{-2}$  mol of dye per mol of silver halide.

50 14. The direct positive silver halide lightsensitive material as claimed in claim 12 wherein the sensitizing amount is within the range of from  $1 \times 10^{-6}$  to  $2 \times 10^{-2}$  mol of dye per mol of silver halide.

\* \* \* \* \*

60

65